# EUROPEAN PATENT SPECIFICATION

(11) **EP 1 598 173 B1**
(45) Date of publication and mention of the grant of the patent: **07.02.2007**
(21) Application number: 05010648.3
(22) Date of filing: 17.05.2005
(51) Int. Cl.: B30B 7/04, B22F 1/00, B22F 3/10

(54) **A method of production of diamond inserts**
Verfahren zur Herstellung von Diamant enthaltenden Metalleinsätzen
Procédé de fabrication d'un insert contenant du diamant

(30) Priority: 18.05.2004 IT TO20040328
(43) Date of publication of application: 23.11.2005
(73) Proprietor: Mimitalia S.r.l., 17047 Vado Ligure (Savona) (IT)
(72) Inventor: Risso, Luca, 16155 Genova (IT)
(74) Representative: Buzzi, Franco

(56) References cited:
- US-A- 5 330 701
- US-A1- 2002 178 862
- US-B1- 6 497 727

## Description

### Field of the invention

The present invention relates to diamond tools, and more in particular:
- to diamond inserts for wires used for cutting blocks in marble and granite quarries, as well as for the production of plates and for cutting concrete in interventions in the sector of conservation building works; and
- to diamond segments and more in general to any sintered diamond abrasive component, especially if it is one of a complex shape.

### State of the prior art

Traditionally, the technologies of production of diamond inserts of which the diamond wire is constituted consist in dry pressing of a mixture of metal dusts - typically Co, Fe, WC, W, Cu, Sn - and diamond granules in dies made of steel or hard metal, followed by sintering. On the other hand, hot-pressing systems using sintering machines are being abandoned on account of the fact that they are far from economically viable.

The starting compositions are constituted by a mixture with variable formulation made up of:
1) fine metal dust, normally having a diameter of between 1 µm and 10 µm, amongst which, for example but not exclusively, Ni, Cu, Fe, Sn, and Zn;
2) a metal binder, usually cobalt;
3) coarse granules of industrial synthetic diamond; and
4) granules of abrasive or reinforcing material (for example, but not exclusively, SiO₂, WC, WC/W₂C, B₄C, SiC, TiC, Mo₂C, CrC, Al₂O₃, in grain sizes up to 250 µm).

The high pressures linked to the friction between the mixture of dusts and the parts of the die, as well as between the different parts of the die themselves, reached during forming of the dusts, usually bring about onset of defects due to the heterogeneity of the mixture and hence of the distribution of the stresses in the die. This is true, in particular, in the step of extraction after compression (formation of cracks and chips). Furthermore, the distribution of the pressure within the die is inhomogeneous, since it is substantially higher in the proximity of the point of contact between the mixture and the force plug (i.e., the part of the die that exerts the force of compression). The traditional technology of compression with cold dies limits the possibility of producing diamond tools with substantially simple shapes. Another drawback related to said conventional technologies is linked to the presence of the diamond, which exerts a considerable abrasive action on the dies, causing fast wear thereof.

The US patent application No. US-2002/0178862 divulges the application of technologies such as metal injection moulding (MIM) to the production of dies made of an alloy of tungsten-cobalt carbide, envisaging the successive steps of preparation of an alloy of tungsten-cobalt carbide with possible addition of other compounds or elements, mixing with plastic additives, injection moulding with MIM technology, removal of the plastic additives, and finally sintering. The sintering temperatures specifically indicated in the prior document No. US2002/0178862 (up to 1370°C) are not compatible with the production of inserts with diamonds in the form of granules.

### Summary of the invention

A purpose of the present invention is to provide a method of production of diamond elements and inserts that will enable the drawbacks described above to be overcome, i.e., will enable a reduction in the forming pressures of the tools and hence in the wear of the dies, exploiting the advantages of known technologies, such as MIM.

A further purpose of the present invention is to reduce substantially the defectiveness in the moulding step.

Yet a further purpose of the invention consists in guaranteeing a high homogeneity in the distribution of the pressure within the pressed component. Another purpose of the invention is to guarantee the possibility of obtaining even complex shapes.

The above purposes are achieved via a method applied to a mixture of metal dusts and diamond granules comprising the following successive steps:
1) preparation of a starting mixture of metal dusts;
2) plasticizing of the starting mixture of metal dusts by means of addition of plastic additives specific for injection moulding of metal dusts (MIM process);
3) addition of diamond granules with a grain size comprised between 10 µm and 300 µm preferably by means of hot plasticizing, homogenization, cooling, and granulation;
4) injection moulding (MIM) at both high and low pressure of said mixture for obtaining diamond elements of the desired shape;
5) removal of the plastic additives;
6) sintering of the diamond elements; and
7) infiltration of the sintered elements with a eutectic alloy for the elimination of any residual porosities.

Sintering of the diamond elements can be performed at temperatures comprised between 900°C and 1100°C. It is also possible to perform the sintering operations with hot-isostatic-pressing (HIP) or hot-pressing technologies. There may likewise be envisaged a possible further final HIP step.

The preferred formulations of the starting mixture of dusts are listed in the following table:

| | Co (wt%) | Fe (wt%) | WC (wt%) | W (wt%) | Cu (wt%) | Sn (wt%) | Diamond (wt%) |
|---|---|---|---|---|---|---|---|
| Formulation 1 | 10-90 | 10-90 | 0-50 | - | | | 0.5-5 |
| Formulation 2 | 10-90 | 10-90 | 0-50 | 0-50 | | | 0.5-5 |
| Formulation 3 | 10-90 | 10-90 | 0-50 | 0-50 | 0-30 | | 0.5-5 |
| Formulation 4 | 10-90 | 10-90 | 0-50 | 0-50 | 0-30 | 0-30 | 0.5-5 |

The grain size of the dust of Co, Fe, WC, W, Cu and Sn is conveniently comprised between 0.01 µm and 100 µm.

The grain size of the diamond grit is typically comprised between 10 and 200 meshes (meshes according to B.S.I. 1943, Tyler 1910 and US Standard 1940).

The plastic additives used can be chosen, for example, from:
1) thermoplastic mixtures with a base of polyolefins such as: polyethylene, polypropylene, ethylvinyl acetate, wax, stearic acid;
2) water-soluble thermoplastic mixtures with a base of polyvinyl alcohol, cellulose compounds and polysaccharides;
3) polyacetalic thermoplastic mixtures; and
4) thermosetting mixtures.

Mixing of the metal dusts with the plastic additives is a hot mixing process performed, for example, in devices of the double-screw extruder type or double-roller mixer type.

The diamond grit is subsequently added by means of hot plasticizing, homogenization, cooling and granulation.

For this step a planetary mixer with Z-shaped blades or Σ-shaped blades can, for example, be used.

The mixture thus obtained is then injection-moulded using MIM (metal-injection moulding) technology with the following critical parameters: pressure comprised between 1 bar and 1000 bar, and temperature comprised between 50°C and 300°C.

There are thus obtained diamond moulded bodies, which are then subjected to de-waxing, i.e., removal of the plasticizing additive.

De-waxing can, for example, be carried out in different alternative ways:
1) using heat by means of thermal treatment in ovens in a controlled atmosphere or air;
2) using organic solvents, such as alcohol, benzene, cylene, etc., or else aqueous solvents; and
3) by means of catalysis in ovens saturated with nitric acid.

Then the moulded and de-waxed bodies thus obtained undergo sintering.

Sintering is carried out typically in an industrial hydrogen furnace, with characteristic temperatures comprised between 900°C and 1100°C. It is possible also to carry out sintering with HIP or else hot pressing.

The mixture formed by pressing and then sintered is next possibly subjected to infiltration with a Cu/Ag eutectic alloy or another infiltrating alloy for the purpose of filling any possible residual porosities present in the inserts.

The elements or inserts thus obtained (each normally provided with a central metal support) are finally mounted on a metal cable to obtain wires that can be used for cutting blocks in marble and granite quarries, as well as for the production of plates and for cutting concrete in interventions in the sector of conservation building works.

Thanks to the method described, a reduction in the pressures of forming of the tools is possible - and hence in the wear of the dies - as likewise a greater homogeneity is obtained in the density of the green compact formed by pressing and consequently a better homogeneity of the physico-mechanical characteristics of the finished product. It is moreover possible to obtain products even of a complex shape as well as to use conveniently MIM technology for the production of diamond inserts, with evident savings in terms of production costs.

The invention affords said advantages thanks to the peculiarity of the combined steps of the method claimed, said combination presenting as an original way of overcoming technical prejudice up to the present day linked to alleged insurmountable operating difficulties in relation to recourse to MIM technologies for forming the diamond elements.

Of course, the modalities and steps of the method may vary widely with respect to what is described merely by way of example herein, without thereby departing from the scope of the present invention as defined in the ensuing claims. Thus, the application of the invention to diamond inserts for diamond wires for cutting is provided purely as an example. An equally advantageous application may in fact be envisaged for the production of diamond segments, which could be in future the main application, and new shapes that have so far not been produced will be possible thanks to the versatility proper to the MIM process.

## Claims

1. A method of production of diamond elements, such as diamond inserts for wires for cutting and the like, **characterized in that** it comprises the successive steps of:
- preparation of a starting mixture of metal dusts;
- plasticizing of the starting mixture of metal dusts by means of addition of plastic additives specific for injection moulding of metal dusts;
- addition of diamond granules with grain size comprised between 10 µm and 300 µm;
- injection moulding by means of MIM (metal injection moulding) technology of the mixture thus obtained for obtaining diamond elements having the desired shape;
- removal of the plastic additives;
- sintering of the diamond elements thus obtained; and
- infiltration of the sintered elements with a eutectic alloy for elimination of any residual porosities.

2. The method according to Claim 1, in which said starting mixture of metal dusts presents one of the following formulations:
| | Co (wt%) | Fe (wt%) | WC (wt%) | W (wt%) | Cu (wt%) | Sn (wt%) |
|---|---|---|---|---|---|---|
| Formulation 1 | 10-90 | 10-90 | 0-50 | - | | |
| Formulation 2 | 10-90 | 10-90 | 0-50 | 0-50 | | |
| Formulation 3 | 10-90 | 10-90 | 0-50 | 0-50 | 0-30 | |
| Formulation 4 | 10-90 | 10-90 | 0-50 | 0-50 | 0-30 | 0-30 |

3. The method according to Claim 1 or Claim 2, in which the grain size of the original metal dust is comprised between 0.01 µm and 100 µm.

4. The method according to Claim 1, in which the added diamond granules have a weight percentage comprised between 0.5 wt% and 5 wt% of the mixture.

5. The method according to Claim 1, in which the plastic additives are chosen in one of the following classes:
a. thermoplastic mixtures with a base of polyolefins such as: polyethylene, polypropylene, ethylvinyl acetate, wax, stearic acid;
b. water-soluble thermoplastic mixtures with a base of polyvinyl alcohol, cellulose compounds and polysaccharides;
c. polyacetalic thermoplastic mixtures; and
d. thermosetting mixtures.

6. The method according to Claim 1, in which the addition of plastic additives to the mixture of dusts occurs in hot conditions in a double-screw extruder.

7. The method according to Claim 1, in which the addition of plastic additives to the mixture of dusts occurs in hot conditions in a double-roller mixer.

8. The method according to Claim 1, in which the addition of diamond granules occurs by means of a planetary mixer with Z-shaped blades.

9. The method according to Claim 1, in which the addition of diamond granules occurs by means of a planetary mixer with sigma-shaped blades.

10. The method according to Claim 1, in which removal of the plastic additives occurs by heat in a controlled atmosphere or air.

11. The method according to Claim 1, in which removal of the plastic additives occurs using organic solvents.

12. The method according to Claim 1, in which removal of the plastic additives occurs via aqueous solvents.

13. The method according to Claim 1, in which removal of the plastic additives occurs by means of catalysis in ovens saturated with nitric acid or oxalic acid.

14. The method according to Claim 1, in which injection moulding according to the MIM technology occurs with pressures of between 1 bar and 1000 bar.

15. The method according to Claim 1, in which injection moulding according to the MIM technology occurs at temperatures of between 50°C and 300°C.

16. The method according to Claim 1, in which sintering is performed at temperatures of between 900°C and 1000°C.

17. The method according to Claim 1, in which sintering is performed by means of HIP or hot pressing.

18. The method according to Claim 1, in which the infiltration eutectic alloy is a Cu/Ag alloy.

## Patentansprüche

1. Verfahren zum Herstellen von Diamantelementen wie Diamanteinsätzen für Schneiddrähte und dergleichen, **dadurch gekennzeichnet, dass** es die nachfolgenden Schritte aufweist:
- Herstellen einer Ausgangsmischung von Metallstäuben;
- Plastifizieren der Ausgangsmischung von Metallstäuben mit Hilfe des Hinzufügens von Kunstharzadditiven, spezifisch für das Spritzgießen von Metallstäuben;
- Hinzufügen von Diamantkörnerchen mit einer Korngröße zwischen 10 µm und 300 µm;
- Spritzgießen mit Hilfe der MIM (Metallspritzgieß)-Technologie der so erhaltenen Mischung zum Erzielen von Diamantelementen mit der gewünschten Form;
- Entfernen der Kunstharzadditive;
- Sintern der so erhaltenen Diamantelemente; und
- Tränken der gesinterten Elemente mit einer eutektischen Legierung zum Entfernen von verbleibenden Porositäten.

2. Verfahren nach Anspruch 1, bei welchem die Ausgangsmischung von Metallstäuben eine der folgenden Mischungen hat:
| | Co (Gew.-%) | Fe (Gew.-%) | WC (Gew.-%) | W (Gew.-%) | Cu (Gew.-%) | Sn (Gew.-%) |
|---|---|---|---|---|---|---|
| Mischung 1 | 10-90 | 10-90 | 0-50 | - | | |
| Mischung 2 | 10-90 | 10-90 | 0-50 | 0-50 | | |
| Mischung 3 | 10-90 | 10-90 | 0-50 | 0-50 | 0-30 | |
| Mischung 4 | 10-90 | 10-90 | 0-50 | 0-50 | 0-30 | 0-30 |

3. Verfahren nach Anspruch 1 oder 2, bei welchem die Korngröße des Ausgangsmetallstaubs zwischen 0,1 µm und 100 µm ist.

4. Verfahren nach Anspruch 1, bei welchem die hinzugefügten Diamantkörnerchen einen Anteil zwischen 0,5 und 5 Gew.-% der Mischung haben.

5. Verfahren nach Anspruch 1, bei welchem die Kunstharzadditive ausgewählt sind aus einer der nachfolgenden Klassen:
a. thermoplastische Mischungen mit einer Basis von Polyolefinen wie: Polyethylen, Polypropylen, Ethylvinylacetat, Wachs, Stearinsäure;
b. wasserlösliche thermoplastische Mischungen mit einer Basis von Polyvinylalkohol, Zelluloseverbindungen und Polysacchariden;
c. polyacetalische thermoplastische Mischungen; und
d. aushärtbare Mischungen.

6. Verfahren nach Anspruch 1, bei welchem das Hinzufügen der Kunstharzadditive zu der Mischung von Stäuben in heißen Zuständen in einem Doppelschraubenextruder erfolgt.

7. Verfahren nach Anspruch 1, bei welchem das Hinzufügen der Kunstharzadditive zu der Mischung von Stäuben in heißen Zuständen in einem Doppelrollenmischer erfolgt.

8. Verfahren nach Anspruch 1, bei welchem das Hinzufügen von Diamantkörnerchen mit Hilfe eines Planetenmischers mit Z-förmigen Schaufeln erfolgt.

9. Verfahren nach Anspruch 1, bei welchem das Hinzufügen von Diamantkörnerchen mit Hilfe eines Planetenmischers mit sigmaförmigen Schaufeln erfolgt.

10. Verfahren nach Anspruch 1, bei welchem das Entfernen der Kunstharzadditive durch Wärme in einer kontrollierten Atmosphäre oder Luft erfolgt.

11. Verfahren nach Anspruch 1, bei welchem das Entfernen der Kunstharzadditive unter Verwendung von organischen Lösungsmitteln erfolgt.

12. Verfahren nach Anspruch 1, bei welchem das Entfernen der Kunstharzadditive mit Hilfe von wässrigen Lösungsmitteln erfolgt.

13. Verfahren nach Anspruch 1, bei welchem das Entfernen der Kunstharzadditive mit Hilfe einer Katalyse in Öfen, gesättigt mit Salzpetersäure oder Oxalsäure, erfolgt.

14. Verfahren nach Anspruch 1, bei welchem Spritzgießen gemäß der MIM-Technologie mit Drücken zwischen 1 bar und 1000 bar erfolgt.

15. Verfahren nach Anspruch 1, bei welchem Spritzgießen gemäß der MIM-Technologie bei Temperaturen zwischen 50° C und 300° C erfolgt.

16. Verfahren nach Anspruch 1, bei welchem das Sintern bei Temperaturen zwischen 900° C und 1000° C durchgeführt wird.

17. Verfahren nach Anspruch 1, bei welchem das Sintern mit Hilfe isostatischen Heißpressens oder Heißpressens erfolgt.

18. Verfahren nach Anspruch 1, bei welchem die eutektische Legierung des Tränkens eine Kupfer/Silber-Legierung ist.

## Revendications

1. Procédé de production d'éléments à base de diamant, tels que des inserts à base de diamant pour des fils à couper et analogues, **caractérisé en ce qu'**il comprend les étapes successives suivantes :
- préparation d'un mélange de départ de poussières métalliques;
- plastification du mélange de départ de poussières métalliques par ajout d'additifs plastiques spécifiques pour un moulage à injection de poussières métalliques ;
- ajout des granules de diamant ayant une granulométrie comprise entre 10 µm et 300 µm;
- moulage par injection, en utilisant la technologie de moulage par injection de métal (MIM) du mélange obtenu pour ainsi obtenir des éléments à base de diamant ayant la forme recherchée ;
- élimination des additifs plastiques ;
- frittage des éléments à base de diamant ainsi obtenus ; et
- infiltration des éléments frittés avec un alliage eutectique pour l'élimination des porosités résiduelles.

2. Procédé selon la revendication 1, dans lequel ledit mélange de départ des poussières métalliques présente l'une quelconque des formulations suivantes :
| | Co (% en poids) | Fe (% en poids) | WC (% en poids) | W (% en poids) | Cu (% en poids) | Sn (% en poids) |
|---|---|---|---|---|---|---|
| Formulation 1 | 10 à 90 | 10 à 90 | 0 à 50 | - | | |
| Formulation 2 | 10 à 90 | 10 à 90 | 0 à 50 | 0 à 50 | | |
| Formulation 3 | 10 à 90 | 10 à 90 | 0 à 50 | 0 à 50 | 0 à 30 | |
| Formulation 4 | 10 à 90 | 10 à 90 | 0 à 50 | 0 à 50 | 0 à 30 | 0 à 30 |

3. Procédé selon la revendication 1 ou selon la revendication 2, dans lequel la granulométrie de la poussière métallique initiale est comprise entre 0,01 µm et 100 µm.

4. Procédé selon la revendication 1, dans lequel les granules de diamant ajoutées ont un pourcentage en poids compris entre 0,5 % en poids et 5 % en poids du mélange.

5. Procédé selon la revendication 1, dans lequel les additifs plastiques sont choisis dans l'une des catégories suivantes :
a. les mélanges thermoplastiques avec une base de polyoléfines telles que : le polyéthylène, le polypropylène, l'acétate d'éthylvinyle, une cire, l'acide stéarique ;
b. les mélanges thermoplastiques solubles dans l'eau avec une base d'alcool polyvinylique, des composés de cellulose et des polysaccharides ;
c. les mélanges thermoplastiques polyacétaliques ; et
d. les mélanges thermodurcissables.

6. Procédé selon la revendication 1, dans lequel l'ajout des additifs plastiques au mélange de poussières se produit dans des conditions chaudes dans une extrudeuse à double vis.

7. Procédé selon la revendication 1, dans lequel l'ajout des additifs plastiques au mélange de poussières se produit dans des conditions chaudes dans un mélangeur à deux cylindres.

8. Procédé selon la revendication 1, dans lequel l'ajout des granules de diamant se produit au moyen d'un mélangeur planétaire avec des pales en forme de Z.

9. Procédé selon la revendication 1, dans lequel l'ajout des granules de diamant se produit au moyen d'un mélangeur planétaire avec des pales en forme de Sigma.

10. Procédé selon la revendication 1, dans lequel l'élimination des additifs plastiques se produit par chauffage dans une atmosphère contrôlée ou dans de l'air contrôlé.

11. Procédé selon la revendication 1, dans lequel l'élimination des additifs plastiques se produit au moyen de solvants organiques.

12. Procédé selon la revendication 1, dans lequel l'élimination des additifs plastiques se produit au moyen de solvants aqueux.

13. Procédé selon la revendication 1, dans lequel l'élimination des additifs plastiques se produit par catalyse dans des fours saturés en acide nitrique ou en acide oxalique.

14. Procédé selon la revendication 1, dans lequel le moulage par injection selon la technologie MIM est effectué sous des pressions comprises entre 1 bar et 1000 bars.

15. Procédé selon la revendication 1, dans lequel le moulage par injection selon la technologie MIM est effectué à des températures comprises entre 50°C et 300°C.

16. Procédé selon la revendication 1, dans lequel le frittage est réalisé à des températures comprises entre 900°C et 1000°C.

17. Procédé selon la revendication 1, dans lequel le frittage est réalisé par pressage isostatique à chaud HIP ou par pressage à chaud.

18. Procédé selon la revendication 1, dans lequel l'alliage eutectique d'infiltration est un alliage Cu/Ag.
